

# UNITED STATES PATENT OFFICE.

ADOLPH OBSER, OF NEWARK, NEW JERSEY.

## MANUFACTURE OF LEATHER.

1,268,876.

Specification of Letters Patent. Patented June 11, 1918.

No Drawing.

Application filed April 18, 1917. Serial No. 162,929.

To all whom it may concern:

Be it known that I, ADOLPH OBSER, a citizen of the United States, and a resident of Newark, in the county of Essex and State of New Jersey, have invented certain new and useful Improvements in the Manufacture of Leather, of which the following is a specification.

The invention relates to a new process for 10 treating hides or skins for the manufacture of leather, and according to said process hides or skins after having been dehaired and prepared for tanning are subjected to the action of a tan bark liquor which serves 15 to perform what may be considered as a preliminary tanning operation. Thereafter the hides which have been subjected to this preliminary tanning operation—and preferably after being split—are subjected to the 20 action of a pickle or "fiber set" as it may be called. When the hides or splits have been properly pickled they are subjected to a subsequent or final tanning operation in an acid tanning solution containing a metallic salt, 25 such as a salt or salts of chromium. Thereafter the splits are preferably subjected to a suitable solution such as an alkaline solution so as to neutralize the acid in the leather, and thereafter washed. Finally the 30 leather is subjected to a stuffing operation in order that there may be incorporated in the leather such fats as are desired. The leather is also subjected to any other finishing operations which are necessary to render the 35 leather fit for its intended use. A specific manner in which the invention may be performed is as follows:

The raw hides if not already in suitable condition, are made ready for the tanning operation, as by performing a dehairing operation and such other preliminary operations as are necessary. The dehaired hides may or may not have been subjected to a preliminary pickle prior to starting the tanning 45 operation, but it is desirable to use hides as green as possible. The question of whether the hides have been subjected to a preliminary pickle or salting is dependent upon whatever steps have been necessary in order that the hides may reach the tannery in proper condition. The dehaired hides are placed in tan bark liquor or bark tanning

as it is frequently referred to. The preferred manner of doing this is to place the hides in rotating or reciprocating drums so 55 that all portions of each hide will be subjected to the action of the tanning solution within the drums. These drums are frequently referred to by tanners as the "rockers". In tanning cow hides, for example, 60 they are subjected to the action in the tan bark liquor or bark tanning solution for from seven to ten days, dependent more or less upon the thickness of the hide and the strength of the bark tanning solution. In 65 other words, the hides remain in this tanning solution about twenty five per cent. Less time than is required where the hides are to be tanned entirely with the bark tanning solution. The bark tanning solution 70 may be referred to as a preliminary tanning solution, since there is effected in this solution only a preliminary tanning or partial tanning operation. After the hides have been removed from the bark tanning solution, and when a large percentage of the moisture (viz., the tan bark liquor) in the 75 hides has been eliminated, as by running through a wringing machine which would leave the hides damp or wet, they are preferably split four or five times. The splits are then subjected to the action of a pickle or "fiber set". This pickle consists of rock or common salt, Glauber salt and sulfuric acid. For example, for one hundred pounds 80 of split hides there is employed a pickling solution consisting of six pounds of rock or common salt, one pound of Glauber salt, and one half pound of sulfuric acid of sixty six per cent. strength. To this there is 85 added about sixteen gallons of water. The leather resulting from the splits is suitable for upholstery of automobiles and the like. The weight of the hides or splits which are subjected to the pickle is taken when the 90 hides or splits are in what may be considered as a dry pressed condition. In other words, when they are moist but when a large percentage of the moisture has been removed therefrom as by pressure. The split hides remain in this pickle for from one half hour to one hour, dependent upon the thickness of the split. At the end of 95 this period there is added to the pickle a so-

lution which provides the metallic salts whereby a subsequent or final tanning operation can take place. The solution containing these metallic salts may be referred to as the standard or the stock solution which, as the name implies, should be kept on hand where the present invention is employed. This standard or stock solution is made as follows:

10 There is first made a liquor comprising four and two tenths pounds of chrome soda (bichromate of soda)—or the proper amount of a bichromate of potash may be used as the chemical equivalent of the sodium chromate—and two and twenty-five one hundredths pounds of wheat white flour. There is finally slowly added sulfuric acid of sixty six per cent. strength, until four and one-half pounds of acid have been added. The 15 resulting solution is allowed to stand about an hour and a half. After it has stood this length of time it can be kept an indefinite length of time prior to being used. An amount of standard solution which is equal 20 to the amount of standard solution resulting from the amounts of ingredients just specified, is then placed in the pickle that is in the rockers or drums when the splits in the rockers or drums have been subjected 25 to the pickle for the proper length of time, and after the standard solution has been added the split hides are allowed to remain for about four or five hours so that a subsequent or final tanning operation will take 30 place.

35 The amount of materials above designated are the proper amounts for the tanning of one hundred pounds of the dry pressed splits. But it will be obvious that 40 in the actual manufacture of standard solution, large quantities will be made at once and it is quite likely that the standard solution or composition will be sold to the users rather than being made by the users themselves. When the standard solution is mixed 45 with the pickle solution already in the rockers, the resulting mixture is an acid solution containing chromium salts. The splits remain in the subsequent or final tanning solution for about four or five hours during 50 which time the chromium acid or tan liquor is released from the chrome salts in the solution due to the acid contained in the solution or mixture within the rockers. A 55 function of the fiber set liquor is to prevent the bark tanning from burning through the splits. The pickle to which the splits were subjected prior to the final tanning operation just referred to, may be considered as an 60 aqueous solution formed of sodium salts (common salt and Glauber salt) and sulfuric acid.

65 At the end of the subsequent or final tanning operation the tanning liquor within the rockers or drums is withdrawn and water at

approximately 80° F., temperature is supplied to the interior of the rockers or drums and the hides are subjected to a washing action within the drums for a period of about ten minutes.

70 The hides are then subjected for about ten minutes to an alkaline solution so as to counteract the acid remaining in the splits. This alkaline solution is made by adding to water one and a half to two per cent. of borax, soda 75 or any other suitable alkali, that is, one-half to two pounds of alkali per hundred weight of split hides. After the alkali treatment there follows a second washing for about ten minutes so as to remove any portions of the 80 alkali solution, whereby the splits will be left in a neutral condition, that is, neither acid nor alkali. A large portion of the moisture mostly water in the split hides may now be removed as by wringing, or it may 85 be left in the washed split hides, and they are ready to be subjected to the fat liquor or stuffing operation, as this fat treatment is frequently called, whereby the proper fats may be introduced into the hide dependent 90 more or less upon the particular use to which the final leather is intended. The fat solution which is preferably employed is an aqueous solution comprising as a component part thereof salt, cottolene, and what is 95 known in the trade as waterless mioellon. Cottolene is a mixture of fats and cottonseed oil but in place thereof any suitable sulfated grease or oil can be used; as, for example, a grease or oil from neat's foot oil 100 or any heavy vegetable oil, such as castor oil or cottonseed oil. In the fat liquor comprising these ingredients the leather is allowed to remain for about half an hour after which the leathers are removed from the liquor and 105 allowed to dry in any suitable manner, and they are also subjected to any other suitable finishing treatment desired. During the time that the hides or splits are being treated, as in the preliminary tanning operation, the 110 pickle, the subsequent tanning operations, the several washes and the fat supplying or stuffing operations, the hides or splits are being agitated or the containers are being revolved so that all portions of the hides or 115 splits are subjected as uniformly as possible to the solution or liquor in which they are. Many of the operations above described have been described as being performed in the same rockers or set of rockers, this being enabled to be done as by removing the liquors or 120 solutions from the rockers by adding liquor or solutions to the rockers or by substituting other solutions in the rockers. It will be manifest, however, that the invention might 125 be performed by removing the hides or splits being treated from one set of rockers or containers, to subsequent sets in which the required solutions for performing the required steps of the process are contained. It is im- 130

possible, for instance, in the bark tanning operation, to accomplish a uniform tanning or partial tanning of the hides. There will be spots of the hide which will be practically 5 completely tanned while other parts of the same hide or split will be only partially tanned. The subjecting of the hides to the subsequent tanning operation above described results in a very uniform product in that those portions of the hide which are 10 completely tanned by the bark tanning are affected very little by the subsequent tanning, while the subsequent tanning operation aids or effects the completion of the necessary tanning upon the portions which are 15 only partially tanned.

The improvements herein set forth are not limited to the precise method herein shown and described, as the invention may be performed in various ways without departing 20 from the spirit and scope thereof.

What I claim is:—

1. In the manufacture of leather the method which comprises subjecting hides to 25 a preliminary tanning operation in a bark-tanning liquor, thereafter splitting and pickling said hides and subjecting the splits to a subsequent tanning operation in a metallic tanning liquor.

30 2. In the manufacture of leather the method which comprises subjecting a hide to the action of a bark-tanning liquor, subsequently splitting and pickling said hide and subjecting said pickled splits to the 35 action of an acid metallic tanning liquor.

3. In the manufacture of leather the method which comprises subjecting dehaired hides to the application of a bark tanning solution, subsequently splitting the hides 40 and thereafter pickling said splits, subjecting said pickled splits to a subsequent tanning operation by the application of an acid metallic tanning liquor until the tanning is completed, neutralizing the tanned splits by 45 the application of an alkaline solution; and finally washing the splits and dressing the same.

4. In the manufacture of leather the method which comprises subjecting a hide 50 to the effect of a bark-tanning solution so as to partially tan said hide, thereafter splitting said hide, pickling said splits and subjecting said pickled splits to a subsequent tanning operation in an acid chrome tanning liquor, washing the splits, neutralizing 55 any acid remaining in said splits by an alkaline solution, washing the splits so as to remove any remaining alkaline solution and finally finishing the leather.

60 5. In the manufacture of leather the method which comprises subjecting hides to a partial bark tanning, splitting said partially bark-tanned hides, pickling said splits in an aqueous solution containing rock or 65 common salt, Glauber salt and sulfuric acid,

thereafter subjecting said splits to a final tanning operation in a solution comprising said pickle to which there has been added an aqueous solution formed from bichromate of potash or chrome soda, wheat flour and sulfuric acid, washing said tanned splits and finally dressing. 70

6. In the manufacture of leather the method which comprises pickling a partially bark-tanned hide and thereafter subjecting 75 said partially bark tanned pickled hide to a final tanning operation in a solution to which there has been added solution formed by the chemical reaction resulting from bichromate of potash or chrome soda, wheat 80 flour and sulfuric acid in the presence of water.

7. In the manufacture of leather the method comprising subjecting a split from a hide partially tanned by a bark-tanning 85 to the action of a pickle or fiber set in which pickle there is rock or common salt, Glauber salt and an acid, subjecting said pickled split to a final tanning by the adding to said pickle a solution or mixture formed from 90 a metallic base and an acid, subjecting the tanned splits to an aqueous alkaline solution, subsequently washing said splits and thereafter subjecting said splits to the action of a fat liquor. 95

8. In the manufacture of leather the method which comprises taking a pickled split which is partially tanned by a bark-tanning liquor the pickling for which was performed after the partial bark-tanning 100 operation and subjecting said pickled split to a final tanning operation in an aqueous solution formed of rock or common salt, Glauber salt and sulfuric acid to which there has been added a stock solution formed 105 of a water-paste comprising bichromate of potash or chrome soda and wheat flour and to which paste there has been added sulfuric acid, allowing the splits to remain in the mixture or solution resulting from the 110 adding of the stock solution to the pickle until the tanning is completed, thereafter neutralizing the effect of the acid in the splits and finishing.

9. A solution for use in tanning which 115 solution is made by mixing, in water, approximately 4.20 pounds of chrome soda and approximately 2.25 pounds of wheat white flour and by adding to the mixture sulfuric acid. 120

10. A standard or stock solution for use in tanning which solution is made by combining 4.20 pounds of chrome soda, 2.25 pounds of wheat white flour and 4.50 parts sulfuric acid of 66 per cent. strength. 125

11. The method of making a stock solution for tanning which comprises mixing together, in water, 4.20 pounds of chrome soda and 2.25 pounds of wheat white flour, and by adding slowly to the mixture sulfuric 130

- acid until there is contained in the mixture the amount of sulfuric acid that is equivalent to that contained in 4.5 pounds of acid of 66 per cent. strength.
5. 12. In the tanning of leather the method which comprises subjecting dehaired hides to bark tanning for about 75 per cent. of the period required to effect a complete tanning of the hides by said tanning liquor, splitting the partially tanned hides, pickling the splits in an aqueous solution containing rock or common salt, Glauber salt and sulfuric acid for a period sufficient to set the fiber in the splits, adding to said pickle an aqueous stock solution formed of bichromate of 15 potash or chrome soda mixed with flour and to which sulfuric has been added, allowing the hides to remain in the solution resulting from the pickle and stock solution 20 until completely tanned, thereafter causing the tanned hides and tanning liquor to be separated from each other, washing the tanned splits, subjecting the washed splits to an alkaline solution, and thereafter again 25 washing the splits in water, subjecting the washed splits to a fat liquor and finally finishing the leather.
13. In the manufacture of leather the method which comprises subjecting hides 30 to a bark-tanning solution, splitting the hides, pickling the partially tanned splits in a solution containing sodium salts and an acid, subjecting the pickled splits to a tanning solution formed of sodium salts, an 35 acid, a chrome base, wheat flour and water, subsequently washing the tanned splits and neutralizing the acid therein, and ultimately stuffing the splits.
14. In the tanning of leather a method 40 which comprises subjecting hides to a partial bark-tanning operation, splitting said partially tanned hides, pickling said splits so as to set the fiber therein, subjecting the pickled splits to a subsequent chrome tanning operation, washing and stuffing said 45 hides.
15. In the manufacture of leather the method which comprises a preliminary bark tanning, a mechanical removal of a large 50 percentage of the bark tanning liquor, a pickling, a metallic tanning and a finishing.
16. In the manufacture of leather splits the method which comprises subjecting a hide to a preliminary bark tanning, splitting 55 and pickling the partially bark tanned hide, subjecting the pickled splits to a sub-
- sequent metallic tanning solution and finally finishing the splits.
17. In the manufacture of leather the method which comprises partially tanning 60 hides, splitting the same, pickling the partially tanned splits, subjecting the pickled partially tanned splits to the action of a chrome tanning solution, washing the tanned splits and subjecting the tanned splits to a 65 fat liquor.
18. In the manufacture of leather splits the method which comprises a preliminary bark tanning operation and a subsequent pickling operation, a subsequent or final tanning operation in a chrome acid tanning solution, neutralizing and washing operations so that no free acid or free alkali will remain in the leather, and a stuffing operation in a fat liquor. 70
19. In the manufacture of leather the method which comprises subjecting a hide to a preliminary tanning operation in a bark-tanning liquor, thereafter splitting said partially tanned hide, subsequently 75 pickling said partially tanned splits, and thereafter subjecting said pickled splits to a tanning operation in a metallic tanning liquor.
20. In the manufacture of leather the 80 method which comprises forming tanned leather splits and subjecting the leather splits to a fat liquor comprising salt, a mixture of fat and cottonseed oil and waterless moellon.
21. An aqueous fat liquor for use in stuffing leather, said liquor comprising salt, a mixture of fat and cottonseed oil and waterless moellon. 85
22. In the manufacture of leather the 90 method which comprises forming tanned leather splits, and subjecting the splits to a fat liquor comprising salt, cottonseed oil or the like and waterless moellon.
23. An aqueous fat liquor for use in stuffing leather said liquor comprising salt, oil and waterless moellon. 100
24. An aqueous fat liquor for use in stuffing leather said liquor comprising salt, cottonseed oil and waterless moellon. 105
- Specification signed and witnessed this 16th day of April A. D., 1917.
- ADOLPH OBSER.
- Signed in the presence of—  
HENRY G. DICKENSHEETS,  
BERFOR OBSER.